

Dec. 31, 1935.

F. H. CONE ET AL

2,026,355

PRODUCTION OF ACTIVATED CARBON

Filed Dec. 17, 1934

Fig. 1.



Fig. 2.



INVENTOR

Frank Henry Cone and  
Elise Buckingham Boulder  
by their atty  
Byrnes, Stebbins & Blenko

## UNITED STATES PATENT OFFICE

2,026,355

## PRODUCTION OF ACTIVATED CARBON

Frank Henry Cone, Southgate, London, and  
Clive Beckingham Houlder, Herts, England,  
assignors to Activities Limited, Nottingham-  
shire, England, a British company

Application December 17, 1934, Serial No. 757,762  
In Great Britain June 24, 1933

7 Claims. (Cl. 252—3)

The present invention relates to the production of activated carbon, for example decolorizing carbon, from such carbonaceous material as will evolve gases when heated, such for example as bituminous coal, lignite, peat or wood in finely divided condition. The term "carbonaceous material" as hereinafter employed refers to such material.

It has previously been proposed to utilize such carbonaceous material in the production of activated carbon by partially burning the material in a powdered condition in a retort in a limited quantity of air at a temperature of the order of 800° C. to 1000° C., and thereafter maintaining the partially burnt material in suspension in the products of its own combustion until activated.

The present invention comprises a process for the production of activated carbon (for example decolorizing carbon) wherein carbonaceous material of the kind described in a finely divided condition (for example bituminous coal in powdered form) is instantaneously raised to a temperature exceeding 1000° C. (for example 1400° C.) by sudden introduction into a zone of incandescent gas so as to decompose it into carbon and hydrocarbons in a fraction of a second. The carbonaceous material is by this means practically instantaneously decomposed without the formation of coke, or contamination of the surface of the carbon particles. A porous and highly active carbon residue is the immediate result. Thus the extended oxidation by gases required to activate the material in other processes becomes unnecessary, and more economical raw materials containing a high proportion of carbon, such as bituminous coal, may be successfully used. It is on this very rapid action that the present invention depends, and the period of activation desirable according to the present invention is generally a very small fraction of a second, say one-hundredth of a second. The more readily a coal forms coke on heating the shorter must be the period allowed for activation without forming coke according to the present invention.

The carbonaceous material may be introduced into a flame of a premixed gaseous fuel and air (for example is carried into the flame in suspension in a mixture of gas and air). The gaseous fuel may be ordinary town gas, having, for example, an approximate analysis comprising 71% hydrogen, 25% carbon monoxide, 2.5% methane, 1% other hydro-carbons and the balance being traces of carbon dioxide and nitrogen. Producer gas, water gas, oil or spirit vapour such as carburetted gas, (i. e., vaporized gas made

from oils or spirits such as petroleum or benzene) or the like, may also be used. The carbonaceous material, together with the gaseous fuel and air, may be injected through a combustion chamber maintained at a temperature exceeding 1000° C.

A plurality of flames may be employed which are caused to impinge upon one another so as to produce a zone of intense combustion and turbulence in which almost instantaneous decomposition takes place, unaccompanied by shrinkage of the carbon residue, which is left in an activated condition.

After the treatment in the burning flame at a temperature exceeding 1000° C. the activation of the carbonaceous material may be enhanced by maintaining it at a lower temperature (for example 900° C.) for a further period of time after which it can be cooled and separated from the gases.

The invention includes apparatus for activating carbonaceous material comprising in combination a combustion chamber, a plurality of burners opening into the chamber for delivering powdered carbonaceous material, air and a gaseous fuel thereto, the said burners being so arranged that the flame issuing from each burner at high velocity commingles with that or those from an adjacent burner or burners.

Further features of the apparatus are herein-  
after described with reference to the accompany-  
ing drawing, which illustrates, by way of example  
and in a diagrammatic form, one form of appa-  
ratus in accordance with the invention.

In the drawing:—  
Figure 1 is a diagrammatic vertical section,

and  
Figure 2 is a horizontal section through the furnace chamber upon the line 2—2 of Figure 1.  
The apparatus comprises a cylindrical com-  
bustion chamber 11 the walls of which are lined  
with refractory material 12 and which has near  
its upper end four radially disposed burners or  
injection nozzles 13.

The refractory lining 12 may with advantage consist of a material which will resist, as far as possible, reaction with the kinds of ash commonly found in carbonaceous materials, such as coal. Highly inert material such as chromic oxide has been found satisfactory.

The burners 13 are arranged in two pairs, one pair being supplied through branches 33 from a pipe 34, and the other pair through branches 35 from a pipe 36. The branches 33 join one another at a Y junction with the pipe 34 so that

the gases are evenly divided between the two burners and the same applies to the branches 35 where they join the pipe 36. The pipes 34 and 36 are symmetrical and join at a Y junction 37 with a supply passage 38 which is connected to an injector 39. In the injector 39 is an air nozzle 40 which delivers preheated air under pressure into the pipe 38 and there is a down pipe 41 for introducing a mixture of coal gas and pulverized 10 bituminous coal. The pulverized bituminous coal is contained in a hopper 16 and is delivered by a worm 17 into a chamber 15 into which opens a gas supply pipe 19.

The air nozzle 40 draws the bituminous coal 15 and the coal gas through the injector 39 and mixes it with air, the whole mixture being delivered into the pipe 38 and thence distributed through the Y branches uniformly between the four burners 13.

20 The burners 13 are disposed so that the flames issuing from them meet in the centre of the upper portion of the combustion chamber 11 above a neck 14 of refractory material which becomes highly incandescent during the process and 25 serves to increase the rate of combustion. The flames meeting in the centre of the combustion chamber produce a zone of intense turbulence and violent combustion. Owing to the circular form of the combustion chamber the walls reflect the maximum of radiant heat on to the gases 30 in this zone, and the ring 14 further reflects heat thereto.

The nozzles or burners 13 are each provided 35 with a multiple-hole opening which subdivides the gases issuing therefrom into a number of jets and thus shortens the zone of unburnt gas in each flame.

40 The lower portion of the combustion chamber 11, constituting the bulk of its volume, serves to receive the descending activated material and gases and to maintain them at an elevated temperature lower than that of the flames themselves of the burners 13 for the purpose of further activating the material which has already been rendered porous and active by its instantaneous 45 decomposition. If necessary in order to reduce the temperature in the lower portion of the combustion chamber 11 cool gases may be introduced through the pipes 25.

50 The activated material and gases pass downwardly through a heat interchanger 21 through the outer portion of which there is passed air from a fan 22, and the air thus preheated is delivered to a pipe 18 at a temperature which may be of the order of 350° C. The pipe 18 delivers this air to the nozzle 40 of the injector 39.

55 The partially cooled gases and carbonaceous material from the chamber 11 are then delivered into a scrubber tower 23 and sprinkled with water from a rose 45 which water percolates downwardly over broken filling and carries down with it carbon suspended in the rising gases. The carbonaceous material collects on the bottom of the tower 23 and the gases pass away through a flue 65 24. The water in the tower 23 is preferably slightly acidulated for the removal of acid-soluble ash in the carbon. The gases have an appreciable calorific value and they may be used as fuel for any purpose desired.

70 The carbon sludge from the tower 23 may be pumped to filtering apparatus and washed.

75 It will be understood that the amount of air delivered to the burners 13 is adequate to burn the gas introduced through the pipe 19 but not to cause complete combustion of the carbon-

aceous material. Some excess air may be introduced for the purpose of burning volatile matter evolved from the carbonaceous material.

On a semi-commercial scale plant, 800 cub. ft. per hour of town gas was injected together with 5 40 lbs. per hour of powdered coal (capable of passing a sieve having 200 meshes to the lineal inch), fed into an injector by means of a screw conveyor, the injector being fed with air pre-heated to a temperature of about 300° C., under 10 a pressure of approximately 3 lbs. per sq. in. The material was exposed to the high carbonizing temperature of approximately 1400° C. for an extremely short period of time about 1/20th sec., the whole carbonization and activation, including treatment in the lower portion of the retort at a reduced temperature being complete in about 15 one second.

It is found that the carbon produced by this process is of a flocculent and porous nature, giving 20 extremely good filtering properties with no tendency towards clogging.

Advantage may be taken of the excess heat generated in this process, by means of heat-exchanging devices, for subsequent heating and 25 drying operations.

We claim:

1. A process for the activation of carbonaceous material comprising injecting finely divided carbonaceous material into a zone of incandescent 30 gas wherein the material is instantaneously raised to a temperature in the vicinity of 1400° C., so as to decompose the material into carbon and hydrocarbons in a fraction of a second and before oxidation of the carbonaceous material 35 can take place.

2. A process for the activation of bituminous coal comprising injecting the bituminous coal in a powdered form into a zone of incandescent gas wherein the powdered material is instantaneously 40 raised to a temperature in the vicinity of 1400° C. so as to decompose the coal into carbon and hydrocarbons in a fraction of a second and before oxidation of the coal can take place.

3. In the preparation of activated decolorizing 45. carbon, a process consisting in introducing to a reaction zone of incandescent gas, carbonaceous material in powdered form, the temperature of the reaction zone being in the vicinity of 1400° C. and the velocity of the particles of the material to said zone being such as to ensure that the material remains at a temperature too low to effect carbonization until it is fully surrounded by the high temperature gases of the zone and thus to decompose the material into carbon and 55 hydrocarbons in a fraction of a second and before oxidation of the carbonaceous material can take place.

4. A process for the activation of carbonaceous material comprising injecting finely divided carbonaceous material into a flame of pre-mixed 60 gaseous fuel and air wherein the material is instantaneously raised to a temperature in the vicinity of 1400° C. so as to decompose the material into carbon and hydrocarbon in a fraction 65 of a second and before oxidation of the carbonaceous material can take place.

5. A process for the activation of carbonaceous material comprising forming a suspension of powdered carbonaceous material in a mixture of 70 gas and air and injecting the suspended material into a flame of incandescent gas wherein the powdered material is instantaneously raised to a temperature in the vicinity of 1400° C. so as to decompose the material into carbon and hy- 75

drocarbons in a fraction of a second and before oxidation of the carbonaceous material can take place.

6. In the preparation of activated decolourizing carbon, a process consisting in introducing finely divided carbonaceous material into a stream of combustible gases so as to be carried thereby in suspension, injecting the suspended material and gases into a combustion chamber, 10 burning the gases in the chamber to maintain it at a temperature in the vicinity of 1400° C. and regulating the velocity of the particles of the injected material to ensure that the material remains at a temperature too low to effect carbonization until it is fully surrounded by the 15 high temperature gases in the chamber and thus decompose the material into carbon and hydrocarbons in a fraction of a second and before oxidation of the carbonaceous material can take place.

7. A process for the activation of carbonaceous material comprising forming a suspension of

finely divided carbonaceous material in a mixture of gaseous fuel and air, injecting the suspended material through a plurality of openings into a combustion chamber, burning the gaseous fuel as it issues from said openings, directing the 5 burning gases to form a plurality of flames which impinge upon one another to produce a zone of intense combustion and a temperature in the vicinity of 1400° C., regulating the velocity of the particles injected into said zone whereby the 10 material is raised instantaneously to a temperature in the vicinity of 1400° C. and thus undergoes carbonization and activation in a fraction of a second, thereafter maintaining the activated material in a further zone at a reduced temperature in the vicinity of 900° C. for a further period of time, the total period of heating in the two 15 zones not exceeding 1 second, cooling the product and separating the gases.

20

FRANK HENRY CONE.  
CLIVE BECKINGHAM HOULDER.